

## UNITED STATES PATENT OFFICE

FREDERICK M. BECKET, OF NEW YORK, N. Y., ASSIGNOR TO ELECTRO METALLURGICAL COMPANY, A CORPORATION OF WEST VIRGINIA

## CORROSION RESISTANT ARTICLES OF MANUFACTURE

No Drawing. Original application filed April 29, 1930, Serial No. 448,428. Divided and this application filed October 29, 1932. Serial No. 640,340.

To increase the resistance of iron to corrosion and to oxidation at elevated temperatures it is customary to incorporate chromium in various quantities. When the chromium content rises to about eighteen per cent or higher with the carbon content suitably low, alloys are produced which have a wide field of application due to their excellent resistance to various corrosive influences. 10 These alloys, however, tend to be deficient in workability and they do not possess the physical properties required to adapt them to severe deep drawing operations.

It has been proposed and has become a common practice to incorporate a content of nickel, for example eight to fifteen per cent, with such a corrosion-resistant iron-chromium base in order to enhance the working properties. This expedient is quite effective 20 for the purpose referred to and the iron-chromium-nickel compositions have gone into extensive use. It has been found, however, that the incorporation of nickel markedly diminishes the ability of the metal to withstand 25 the action of sulphur dioxide, hydrogen sulphide and other sulphur compounds, and in certain applications where sulphur compounds are encountered at elevated temperatures and where a high degree of ductility 30 should be preserved, neither the binary iron-chromium alloy nor the ternary iron-chromium-nickel alloy meets the requirements.

I have found that a high degree of workability can be imparted to corrosion resistant iron-chromium alloys by appropriate additions of manganese and that unlike nickel the manganese does not appear to impair the resistance to corrosion in any respect. In comparative tests the iron-chromium-manganese alloys are found to resist the action of such agents as sulphurous acid and moist hydrogen sulphide at ordinary and elevated temperatures, substantially to the same degree as the most resistant binary chromium 40 irons, and far better than any iron-chromium-nickel alloys which have come to my attention.

The best properties are exhibited by alloys containing from about fifteen to about 50 twenty-two per cent of chromium. To de-

velop the maximum degree of workability I prefer a proportion of manganese within the range embraced between the approximate limits of six per cent and sixteen per cent. More manganese may be added but it will not 55 as a rule bring about an improvement in properties sufficient to warrant the additional expense. The iron-chromium-manganese alloys are discussed in more detail in my application Serial No. 435,957, filed March 14, 1930. As 60 is there stated the workability of the alloy increases as the carbon content is diminished, and where severe working operations are contemplated the carbon content should not be above about three tenths per cent and is preferably below twelve hundredths per cent. 65

The iron-chromium-manganese may be additionally modified by the incorporation of other elements, and without sacrificing its resistance to corrosion by sulphur compounds. 70 Thus I may add copper in proportions from about one-fourth of one per cent up to about three per cent. A substantial addition to copper tends to improve the deep drawing qualities of the alloy as is more fully explained 75 in my application, Serial No. 444,876, filed April 16, 1930. Excessive proportions of copper engender a tendency towards hot shortness. The maximum useful proportion of copper, as is explained in my said prior 80 application, depends in some measure on the proportion of manganese present.

A principal field of application for the herein described alloys is in the thermal decomposition of hydrocarbon material, for 85 example the cracking of petroleum fractions to produce gasoline. Such decompositions are ordinarily carried out in tubes and the latter may be subjected at a high temperature 90 to oxidizing conditions on the outside and simultaneously to the action of sulphur compounds associated with the material being cracked and contained within the tubes. The alloys are in all respects admirably adapted 95 to the fabrication of tubes for such operations, and they are equally suitable for making the tubular condensers in which the cracked products are usually liquefied.

This application is a division of a prior 100

application, Serial Number 448,428, filed April 29, 1930.

I claim:

1. An oil cracking tube composed of a stain-resisting iron-base alloy having deep-drawing properties and containing chromium about 16% to 22%; manganese about 6% to 16%; copper about 0.25% to 2.5%; and carbon, the carbon content being not more than about 0.3%; with the balance substantially iron.

2. An oil cracking tube composed of a stain-resisting iron-base alloy having deep-drawing properties and containing chromium about 16% to 22%; manganese about 6% to 16%; copper about 0.25% to 2.5%; and carbon, the carbon content being not more than about 0.12%; with the balance substantially iron.

20 In testimony whereof, I affix my signature.  
FREDERICK M. BECKET.

25

30

35

40

45

50

55

60

65